

## 1

3,413,397

## PROCESS FOR STRETCHING POLYPROPYLENE FILAMENTS

Robert E. Bierbaum and Emmett V. Martin, Kingsport, Tenn., assignors to Eastman Kodak Company, Rochester, N.Y., a corporation of New Jersey

No Drawing. Continuation-in-part of abandoned application Ser. No. 649,004, Mar. 28, 1957. This application Aug. 17, 1961, Ser. No. 132,017

2 Claims. (Cl. 264—290)

This invention relates to a method for producing polyolefin fibers having improved properties. More particularly this invention relates to a method of stretching polypropylene fibers which have substantially improved tenacity and modulus of elasticity.

This application is a continuation-in-part of our application Ser. No. 649,004, filed Mar. 28, 1957, now abandoned.

In recent years many types of synthetic fibers have been developed. These synthetic fibers as produced do not, a number of times, possess as good properties as may be desired in the fibers. Hence, a number of after-treatment methods and apparatus are described in the art for application to synthetic fibers for the improvement thereof. In general many of these after-treatments involve the application of heat to the fibers.

Numerous devices and media have been suggested for the application of heat as well as physical treatment of yarn. Among these are heated rolls and shoes, high frequency electromagnetic fields, heated liquids and heated gases and vapors. Unless the medium itself, such as a fluid, exerts a swelling or plasticizing action on the yarn, the type of heating medium employed ordinarily exerts little influence on the final properties of the yarn. Therefore, in the prior art the choice of methods of after-treatment has in many instances been made on the basis of convenience or economics.

Polyolefin fibers and yarns have been produced in recent years. While such polyolefin yarns are very resistant not only to water but different chemicals, and possess other useful properties, these polyolefin yarns have certain physical properties which are not as good as may be desired. Hence, it is apparent that the development of a method of treatment of such polyolefin yarns whereby the yarn can be improved, such as in its strength and elasticity, represents a highly desirable result.

After extended investigation we have found that polyolefin yarns, and in particular polypropylene yarn, somewhat in contrast to other synthetic yarns, react differently to different types of after-treatment and are particularly sensitive to a certain type of after-treatment. We have found that if polyolefin yarns of the class described herein are drawn in steam preferably super-heated steam as described in more detail hereinafter by a process employing relatively high draw ratios, that the properties of such polyolefin fibers and yarns are unexpectedly improved. This is unexpected because polyolefin yarns are quite hydrophobic and under ordinary circumstances have heretofore been regarded as little affected by water or water vapor. Use of steam rather than dry heat for the drawing medium results in greatly improved operation of the process. The yarns can be drawn at a greater rate of speed and with fewer broken filaments with use of steam. We have further found, in accordance with a more detailed embodiment of our invention, that if the steam-treated polyolefin yarn as just described is also given a heat treatment (heat-setting treatment) as will be described hereafter, that the yarn is still further improved. That is, by this latter step the polyolefin yarn is stabilized against shrinkage in boiling water.

The improvement obtained by treating polyolefin yarns

## 2

with relatively high draw ratios and in steam in accordance with the present invention, and as will be set forth in detail hereinafter, appears to be considerably greater than can be obtained by after-treatments by other processes which might appear to be somewhat similar or comparable.

This invention has for one object the production of polyolefin fibers having improved properties. A particular object is to provide polypropylene and polyethylene fibers which have enhanced tenacity and modulus of elasticity. Still a further object is to provide a method of treating polyolefin yarns such as polypropylene yarn in a relatively simple, uncomplicated manner which will give improvements in the yarn in relatively few processing steps. Still another object is to provide a method for treating polyolefin yarns with superheated steam, and also in certain instances with heat-setting, which methods employ relatively high draw ratios and gives treated yarn having improved properties. Other objects will appear hereinafter.

As indicated above, in the broader aspects of our invention we have found that polyolefin yarns, even though they are normally quite hydrophobic and little affected by water or water vapor, may be drawn at high draw ratios in a steam atmosphere, particularly a superheated steam. Such drawing at high draw ratios in such steam atmosphere quite unexpectedly permits obtaining yarns having a substantially greater strength and modulus of elasticity than may be accomplished by other types of treatment which may appear comparable. The polyolefin yarns of the present invention may be produced in various ways. These methods in their broader aspects comprise fluidizing polyolefin material such as by melting. Then the melted material is extruded through forming means such as spinnerettes to obtain the filaments, which filaments may be cooled in any conventional manner and wound up on yarn packages. For the purposes of illustration the following brief example will indicate how the polyolefin yarns employed in the present invention were prepared.

Five pounds of the polyolefin, in this instance polypropylene, were placed in the hopper of a melt extrusion apparatus. The polymer was vacuum dried. Following drying, an inert gas was introduced into the hopper to break the vacuum, and this inert atmosphere was then maintained above the polymer. The polypropylene used had a number-average molecular weight of about 75,000 and was of the type known generally in the trade as high molecular weight polypropylene. The hopper feeds into a heated screw mechanism of conventional construction. The polypropylene was heated to a temperature within the range of 200 to 360° C. so that it was readily flowable. The fluid polypropylene was extruded under pressure between 150 p.s.i.g. and 500 p.s.i.g. through a spinnerette nozzle having approximately 50 openings of circular configuration of a diameter of about 0.30 mm.

The polypropylene filaments emerging from the spinnerette were cooled in air by passing down a spinning column about 15 feet long. The cooled polypropylene filaments were gathered on a parallel package winder to form a yarn package containing approximately 1600 yards (0.33 lbs.) of polypropylene.

While we have described the production of 600-900 denier yarn containing about 50 filaments, other size yarn may be made in a similar manner. Likewise in a similar manner and with similar apparatus polyethylene yarn may be produced.

The yarn produced as described above or by some other method, is then ready for an after-treatment in accordance with the present invention for improving its properties. It will be noted that the polyolefin yarn when treated by the present invention, is drawn at relatively high draw ratios, say a draw ratio in excess of four. The drawing

equipment employed in the present invention consists of a feed roll. This roll is merely a means for withdrawing the end of the yarn from the yarn package and feeding it into the process. Means are provided for heating the yarn, usually referred to as drawing medium. This medium in accordance with the present invention is steam. However, it will be noted in the description which follows that reference will be made to employing either heated air or a heated roll in order to provide data for comparison with the use of steam in accordance with the present invention, from which it may be seen that operating with steam in accordance with the present invention gives improved results.

Finally, in the apparatus there is a draw or take-up roll. The yarn passes in the undrawn state from the yarn package to the feed roll from which the yarn is fed at a reasonably steady rate. The yarn then passes over or through the drawing medium which, as indicated in the present invention is steam. Then while the yarn is in a steam treated condition it is drawn many times its original length by means of the take-up or draw roll. The treated yarn from the draw roll is then repackaged in any convenient manner. As already mentioned, it will be noted from the present invention that the draw roll is operated at relatively high

In the examples which follow the yarn feed speed was 15-30 feet per minute. The steam chamber used was approximately 24" long, supplied with steam at the desired rate through a preheater and a conventional pressure or flow regulating device. The yarn from the feed roll was threaded through a narrow slot on three sides of the steam chamber.

In the instance where the runs were carried out on a heated roll, the heated roll was a small internally heated metal roll which revolves with a surface speed equal to the 10 yarn feed speed. The yarn was in contact with the heated roll for the various lengths specified in the runs. Roll temperature was measured by a surface temperature pyrometer.

In the runs where hot air was employed as the heating medium, the hot air chamber was made from a 2" diameter cylindrical rod about 18" long. An axial slot  $\frac{1}{8}$ " wide and 1" deep was cut in the rod. The yarn ran through this slot. The rod was heated by electrical cartridge type 20 heaters. The temperature listed in the runs is the temperature of the rod which is an approximate measure of the air temperature.

With the above description of apparatus in mind, attention may now be turned to the following examples:

EXAMPLE I.—EXAMPLES OF DRAWING CRYSTALLINE POLYPROPYLENE

| Run No. | Drawing medium                 | Draw ratio | Tenacity, g./den. | Elongation, percent | Modulus of elasticity, g./den. |
|---------|--------------------------------|------------|-------------------|---------------------|--------------------------------|
| 1.....  | Superheated steam at 165° C... | 9.5        | 6.2               | 14                  | 60                             |
| 2.....  | Air at 165° C.....             | 10.5       | 5.5               | 11                  | 50                             |
| 3.....  | Superheated steam at 120° C... | 9.5        | 7.0               | 16                  | 75                             |
| 4.....  | Air at 120° C.....             | 10.0       | 6.9               | 14                  | 76                             |
| 5.....  | Hot roll at 120° C.....        | 9.5        | 5.3               | 12                  | 75                             |

EXAMPLE II.—EXAMPLES OF DRAWING HIGH DENSITY POLYETHYLENE

| Run No. | Drawing medium                                      | Draw ratio | Tenacity, g./den. | Elongation, percent | Modulus of elasticity, g./den. |
|---------|-----------------------------------------------------|------------|-------------------|---------------------|--------------------------------|
| 1.....  | Steam at 105° C.....                                | 18.0       | 5.85              | 5                   | 144                            |
| 2.....  | Heated roll at 85° C., $2\frac{1}{2}$ in. contact.  | 7.6        | 3.83              | 18                  | 40                             |
| 3.....  | Heated roll at 105° C., $2\frac{1}{2}$ in. contact. | 8.0        | 4.90              | 17                  | 53                             |
| 4.....  | Heated roll at 105° C., $\frac{1}{2}$ in. contact.  | 8.66       | 4.95              | 17                  | 48                             |
| 5.....  | Hot air, chamber temp. 110° C.                      | 7.40       | 3.52              | 19                  | 43                             |
| 6.....  | Hot air, chamber temp. 120° C.                      | 7.72       | 4.52              | 21                  | 41                             |

EXAMPLE III

| Run No. | Drawing medium                                      | Draw ratio | Tenacity, g./den. | Elongation, percent | Modulus of elasticity, g./den. |
|---------|-----------------------------------------------------|------------|-------------------|---------------------|--------------------------------|
| 1.....  | Steam at 105° C.....                                | 14.4       | 5.90              | 9                   | 115                            |
| 2.....  | Heated roll at 85° C., $2\frac{1}{2}$ in. contact.  | 9.3        | 3.72              | 18                  | 49                             |
| 3.....  | Heated roll at 105° C., $2\frac{1}{2}$ in. contact. | 9.5        | 3.78              | 18                  | 40                             |
| 4.....  | Heated roll at 105° C., $\frac{1}{2}$ in. contact.  | 7.7        | 3.03              | 20                  | 33                             |
| 5.....  | Hot air, chamber temp. 113° C.                      | 8.8        | 3.76              | 17                  | 43                             |
| 6.....  | Hot air, chamber temp. 134° C.                      | 9.3        | 4.32              | 17                  | 47                             |

speed compared with the feed roll in order that a somewhat higher draw ratio is applied to the polyolefin yarn undergoing treatment by the steam process of the present invention.

The present invention will be further understood from the following examples which will be set forth. In these examples it will be noted that the first runs are illustrations of treatment in accordance with the present invention. Certain of the other runs are illustrations of prior art methods such as rather than using steam using hot air, heated rolls, etc. From these other runs it is possible to compare the results and observe the improvement obtained by the method of the present invention which employs steam.

In the above examples draw ratio means the number obtained by dividing the surface speed of the draw roll by the surface speed of the feed roll. The tenacity, elongation, and modulus of elasticity were measured on a standard Instron tensile tester with an elongation rate of 100% per minute. The modulus of elasticity is the slope of the initial straight portion of the stress-strain curve, expressed in grams per denier per unit extension.

It is believed apparent from the preceding examples that it can be seen by using the relatively high draw ratios of 4 and in some instances above 8, in combination with steam that the properties of the polyolefin yarn are considerably improved over properties obtained by other methods of comparable simplicity and economy. For poly-

propylene yarn we would generally prefer steam at between 120° C. and 165° C. In general superheated steam is preferred for all types of polyolefin yarn, but saturated steam can also be used.

From the foregoing it will be seen that we have shown a method for improving the tenacity and modulus of yarns consisting of polypropylene and polyethylene. We have further found that there may be coupled with the treatment which has been described above a heat-setting step whereby the polyolefins of the class indicated may be stabilized against shrinkage in boiling water.

In further detail, this stabilization against boiling water shrinkage can be accomplished by heat-setting the polyolefin yarn in hot air on a heated roll or shoe or in steam. The yarn can be held at constant length or allowed to shrink during the treatment.

For polypropylene yarn we have found the range of temperatures useful for this heat-setting purpose is from about 90° C. to 140° C. and the time from 5 seconds to 5 minutes. Temperatures below 90° C. are substantially ineffective and the use of temperatures above 140° C. may result in the filaments adhering to each other and the loss of properties. Treatment for times less than 5 seconds produces rather little effect and the use of times longer than 5 minutes appears to be unnecessary.

In the case of the high density polyethylene yarns, the preferred temperature range is from about 90° C. to 120° C. and the time range from 5 seconds to 5 minutes.

This embodiment of our invention pertaining to heat-setting will be further illustrated by the several examples which follow:

**EXAMPLE IV.—EXAMPLE OF HEAT-SETTING POLYPROPYLENE YARN IN HOT AIR WHILE HELD AT CONSTANT LENGTH**

| Temperature, °C. | Time    | Tenacity (g./d.) | Elongation, percent | Shrinkage in boiling water, percent |
|------------------|---------|------------------|---------------------|-------------------------------------|
| Control          |         | 5.6              | 36                  | 8.5                                 |
| 100              | 30 sec. | 6.0              | 33                  | 6                                   |
| 100              | 5 min.  | 6.2              | 38                  | 3.8                                 |
| 130              | 10 sec. | 6.0              | 40                  | 4                                   |
| 130              | 30 sec. | 6.0              | 45                  | 2                                   |
| 130              | 5 min.  | 5.3              | 35                  | 1.5                                 |

**EXAMPLE V.—EXAMPLE OF HEAT-SETTING HIGH DENSITY POLYETHYLENE YARN IN HOT AIR WHILE HELD AT CONSTANT LENGTH**

| Temperature, °C. | Time    | Tenacity (g./d.) | Elongation, percent | Shrinkage in boiling water, percent |
|------------------|---------|------------------|---------------------|-------------------------------------|
| Control          |         | 4.3              | 19                  | 8.3                                 |
| 100              | 30 sec. | 4.4              | 19                  | 6.2                                 |
| 100              | 5 min.  | 4.5              | 21                  | 3.2                                 |
| 115              | 5 sec.  | 4.5              | 20                  | 4.6                                 |
| 115              | 30 sec. | 4.6              | 23                  | 2.7                                 |
| 115              | 5 min.  | 4.6              | 23                  | 1.4                                 |

**EXAMPLE VI.—EXAMPLE OF HEAT-SETTING POLYPROPYLENE YARN IN HOT AIR WITHOUT CONSTRAINT**

| Temperature, °C. | Time    | Shrinkage during heat-setting |                   | After heat-setting |                                     |
|------------------|---------|-------------------------------|-------------------|--------------------|-------------------------------------|
|                  |         | percent                       | Tenacity, (g./d.) | percent            | Shrinkage in boiling water, percent |
| Control          |         | 5.6                           | 36                | 8.5                |                                     |
| 100              | 30 sec. | 8                             | 4.9               | 40                 | 0.7                                 |
| 100              | 5 min.  | 10.2                          | 4.8               | 41                 | 0                                   |
| 130              | 30 sec. | 17                            | 4.3               | 62                 | 0                                   |
| 130              | 5 min.  | 33                            | 3.0               | 60                 | 0                                   |

**EXAMPLE VII.—EXAMPLE OF HEAT-SETTING HIGH DENSITY POLYETHYLENE YARN IN HOT AIR WITHOUT CONSTRAINT**

| Temperature, °C. | Time    | Shrinkage during heat-setting |                   | After heat-setting |                                     |
|------------------|---------|-------------------------------|-------------------|--------------------|-------------------------------------|
|                  |         | percent                       | Tenacity, (g./d.) | percent            | Shrinkage in boiling water, percent |
| Control          |         | 4.3                           | 19                | 8.3                |                                     |
| 100              | 30 sec. | 9.6                           | 3.2               | 32                 | 0                                   |
| 100              | 5 min.  | 10.5                          | 3.2               | 32                 | 0                                   |
| 115              | 30 sec. | 33                            | 2.1               | 111                | 0                                   |
| 115              | 5 min.  | 33                            | 2.1               | 89                 | 0                                   |

While we have described in particular the treatment of 50 filament 600-900 denier yarn in the above examples, our invention may be applied to other sizes of yarn which are useful in the textile industry. The composition of the above yarns was substantially 100% polyolefin. We regard it as surprising that a polyolefin yarn which will absorb practically no water, will respond in such a striking fashion, as set forth above, to the use of steam as a medium for drawing. However, polyolefin yarns of slightly modified compositions can be similarly treated. For example, polyolefin yarns containing relatively small amounts of modifiers such as dyes, pigments, ultraviolet inhibitors, antioxidants, plasticizers, fillers, and even copolymerizable compounds to an extent in most cases not more than 5% and in no case more than 10% by weight of the polyolefin can be processed in a comparable manner to obtain improved yarn products. The number-average molecular weight of the polyolefin will usually be above 5,000 and below 200,000, and preferably will be within the range of 10,000 to 50,000.

The invention has been described in considerable detail with particular reference to certain preferred embodiments thereof, but it will be understood that variations and modification can be effected within the spirit and scope of the invention as described hereinabove, and as defined in the appended claims.

We claim:

1. A process for treating polypropylene filamentary material having a molecular weight of at least 5,000 and including:
  - 35 drawing said filamentary material to at least four times its original undrawn length in an atmosphere of steam at a temperature of at least about 100° C.; and thereafter
  - heat-setting said filamentary material in a hot gaseous atmosphere at a temperature of from between about 120° C. and the melting point of said filamentary material.
2. A process in accordance with claim 1 wherein steam is superheated and is at a temperature of at least about 120° C.

**References Cited**

**UNITED STATES PATENTS**

- 45 2,360,352 10/1944 Lodge ----- 8—151.2
- 2,371,579 3/1945 Cole et al. ----- 8—132
- 2,437,263 3/1948 Manning ----- 264—210 X
- 2,468,081 4/1949 Koster.
- 2,586,800 2/1952 Elvin et al.
- 2,584,043 1/1952 Oberley.
- 2,622,961 12/1952 Finlayson et al.
- 2,661,618 12/1953 Bessom.
- 2,664,010 12/1953 Emerson.
- 3,173,977 3/1965 Esselmann et al. ----- 264—210
- 2,325,060 7/1943 Ingwersoll ----- 28—1
- 2,411,474 11/1946 Stevenson ----- 28—1
- 2,420,565 5/1947 Rugeley et al. ----- 28—1
- 2,821,457 1/1958 Erlich ----- 28—1
- 2,953,428 9/1960 Hunt et al. ----- 8—130 X
- 2,956,330 10/1960 Pitzl ----- 28—78
- 2,289,860 7/1942 Babcock ----- 264—232
- 2,390,132 12/1945 Smith et al. ----- 28—1
- 2,596,128 5/1952 Chavannes et al. ----- 264—290
- 2,679,450 5/1954 Hampson et al. ----- 264—206
- 65 2,934,400 4/1960 Sigel et al. ----- 264—210

**OTHER REFERENCES**

Handbook of Chemistry and Physics, 39th ed., pub. by Chemical Rubber Pub. Co., Cleveland, Ohio, pp. 2262, 2270, 2272, 2274, 1957-58.

70 Hill, Fibres from Synthetic Polymers, Elsevier Pub. Co., New York, 1953, pp. 6, 47.

JULIUS FROME, Primary Examiner.

J. H. WOO, Assistant Examiner.